# EUROPEAN PATENT APPLICATION

(11) **EP 4 782 562 A1**
(43) Date of publication of application: **29.07.2026**
(21) Application number: 24884601.6
(22) Date of filing: 25.10.2024
(51) Int. Cl.: C22C 21/04, C22C 1/02, C22C 1/03

(54) **HEAT TREATMENT-FREE HIGH-STRENGTH AND HIGH TOUGHNESS DIE-CASTING ALUMINUM ALLOY, PRODUCT PREPARED THEREFROM, AND PREPARATION METHOD THEREFOR**

(30) Priority: 31.10.2023 CN 202311425104
(71) Applicant: BAOSHAN IRON & STEEL CO., LTD., Shanghai 201900 (CN)
(72) Inventor: LIU, Jinyan, Shanghai 201900 (CN); ZENG, Yu, Shanghai 201900 (CN); WU, Chang, Shanghai 201900 (CN); XUE, Fei, Shanghai 201900 (CN); YANG, Bing, Shanghai 201900 (CN)
(74) Representative: Maiwald GmbH
(86) International application number: PCT/CN2024/127391
(87) International publication number: WO 2025/092598

(57) **Abstract**

The present disclosure relates to a heat-treatment-free high-strength and high-toughness die-cast aluminum alloy, an article prepared therefrom and a manufacturing method therefor. In addition to Al and inevitable impurity elements, the die-cast aluminum alloy comprises the following chemical components in percentage by mass: 6.5-9.5% of Si, 0.1-0.3% of Fe, 0.4-0.85% of Mn, 0.1-0.6% of Mg, 0.1-0.9% of Cu, 0.02-0.12% of Ti and 0.05-0.15% of Sb; and satisfies the following formulas: Fe+Mn ≥ 0.65%; and Mn/Fe = 2.0-6.6, wherein each element symbol is substituted with the content of the corresponding element in percentage by mass. The disclosure solves the problem of unstable elongation due to melt gas absorption caused by Sr modification in such heat-treatment-free die-cast alloys, enabling the aluminum alloy die-cast part to obtain a microstructure without obvious porosity and shrinkage defects throughout the interior, thereby ensuring a tensile strength of greater than 230 MPa, a yield strength of greater than 150 MPa, and an elongation of greater than 10% at various portions of the part.

## Description

### TECHNICAL FIELD

The present disclosure relates to the technical field of die-cast aluminum alloy, and in particular to a heat-treatment-free high-strength and high-toughness die-cast aluminum alloy, an article manufactured therefrom and a manufacturing method therefor.

### BACKGROUND ART

The development of the modern automobile industry has driven the demand for high-strength and high-toughness die-cast aluminum alloy. Since the 1990s, researchers domestic and abroad have been committed to developing high-strength and high-toughness die-cast aluminum alloy material on the basis of high-vacuum die-casting technology, mainly focusing on Al-Si-Mg-based alloy (a typical alloy composition is AlSi10MnMg). This is because Mg and Si in the Al-Si-Mg alloy can form Mg₂Si, which can solid-solutionize into the matrix during heat treatment and subsequently precipitate during aging to strengthen the alloy. At the same time, Si particles can be spheroidized and passivated during solid solution, thereby improving the plasticity of the alloy.

To meet the requirement of high elongation performance, traditional aluminum die-cast body components typically require heat treatment. However, as the size of integrated castings becomes larger, deformation is prone to occur during heat treatment, resulting in a decrease in the yield rate. Therefore, heat-treatment-free material has become the best choice in the implementation of integrated die-casting technology. The required as-cast tensile mechanical properties of large integrated thin-walled parts are as follows: yield strength ≥ 120 MPa, tensile strength ≥ 200 MPa, and elongation ≥ 10%. In view of the inadequate performance of the conventional die-cast aluminum alloys without heat treatment, several manufacturers or research institutions have disclosed prior art for heat-treatment-free die-cast aluminum alloys.

Chinese publication with Publication No. CN115505795A discloses a heat-treatment-free aluminum alloy material, which includes the following components: Si, Fe, Cu, Mn, Mg, Zn, Ti, Sr, Zr, Cr, B, rare earth elements La+Y, Al and inevitable impurity elements. The components are formulated in the following in percentage by mass: 7.0-10.5% of Si, 0.1-0.8% of Fe, 0.95-4.0% of Cu, 0.2-0.7% of Mn, 0.4-1.44% of Mg, 0.1-1.2% of Zn, 0.036-0.1% of Ti, 0.02-0.06% of Sr, 0.002-0.06% of Zr, 0≤Cr<0.008% of Cr, 0≤B<0.002% of B, 0≤La+Y<0.2% of rare earth elements La+Y, the balance being Al and inevitable impurity elements. The advantage of the invention lies in: in terms of composition design, Si is controlled within the range of 7-10% in the hypoeutectic series, which can effectively improve the fluidity and filling capacity of the aluminum alloy. Through the synergistic effect with other elements, the yield strength is improved while ensuring a certain elongation, and the grain size of the die-cast structural casting is significantly refined, achieving a dual refinement effect.

Chinese publication with Publication No. CN115094281A discloses a heat-treatment-free bake-hardenable die-cast Al-Si alloy, a manufacturing method and a bake-hardening method. The die-cast aluminum alloy comprises the following elements in percentage by mass: 5.5-8.0% of Si, 0.2-0.9% of Mg, 0.1-0.6% of Cu, Fe≤0.2%, Mn≤0.4%, Mo≤0.4%, Ni≤0.1%, Sn≤0.1%, Ti≤0.1%, 0.01-0.02% of Sr, the balance being Al and inevitable impurities, wherein the mass ratio of Cu element to Mg element is ≤0.65, the mass ratio of Mn element to Mo element is 1.0-2.0, and the mass ratio of the sum of Mn element and Mo element to Fe element is 3.0-6.0. The die-cast Al-Si alloy is manufactured by preparing raw materials, smelting, refining and die casting, and has excellent tensile strength, yield strength and good plasticity without heat treatment.

Chinese publication with Publication No. CN114717455A discloses a heat-treatment-free high-strength and high-toughness die-cast aluminum alloy and a manufacturing method thereof. The alloy includes: 7.5-9.5 wt.% of Si, 0-1.5 wt.% of Ni, 0.4-0.8 wt.% of Mn, 0-0.4 wt.% of Mg, 0.08-0.3 wt.% of Cr, 0.01-0.15 wt.% of Zr, 0.03-0.1 wt.% of Ti, 0.005-0.025 wt.% of Sr, and the balance being aluminum and inevitable impurity elements. The die-cast aluminum alloy of the invention has good thermal stability, so that the change in mechanical properties is not more than 10% after being kept at a temperature not higher than 150 °C for 1000 h, as well as excellent mechanical properties with an as-cast yield strength greater than 120 MPa and an elongation of greater than 14%. The property requirements of die-cast structural component for car bodies can be met without subsequent heat treatment, and the yield rate of thin-walled die-cast structural components can be greatly increased, reducing the cost of automobile parts.

Chinese publication with Publication No. CN114164362A discloses a heat-treatment-free high-strength and high-toughness aluminum alloy and a forming method thereof. The aluminum alloy has the following components in percentage by mass: 8.5-11.5% of Si, 0.05-0.5% of Cu, 0.05-0.5% of Mg, 0.1-0.5% of Mo, 0.005-0.1% of Sr, 0.005-0.1% of B, 0.05-0.3% of Cd, 0.05-0.25% of Zr, and the balance being Al and inevitable impurities. In the forming of the aluminum alloy of the invention, boronization is utilized to refine grains, while strontium modification is used to refine eutectic silicon, and the addition of Mo not only avoids the poisoning phenomenon caused by the simultaneous addition of B and Sr, but also refines the eutectic silicon to a submicron-scale size, greatly improving the strength and toughness of the alloy. Meanwhile, combined with solution strengthening and dispersion strengthening, the alloy is endowed with excellent mechanical properties. The alloy has good fluidity, excellent casting performance, and does not need heat treatment for strengthening, which saves production procedures, reduces production cost and has a bright application prospect.

Chinese publication with Publication No. CN105316542A discloses a high-strength and high-toughness die-cast aluminum alloy and article thereof. The alloy is a Al-Si-Mn-Mg-Re based alloy, and consists of the following components in percentage by mass: 7.5-8.5% of silicon, 0.3-0.4% of manganese, 0.2-0.3% of magnesium, 0.1-0.2% of rare earth, 0.01-0.02% of strontium, Fe≤0.15%, Ti≤0.10%, Cu≤0.05%, and the balance being aluminum and inevitable trace impurities, wherein the content of a single trace impurity element is ≤0.05%, and the total content of trace impurities is ≤0.15%. The article is prepared from the above high-strength and high-toughness die-cast aluminum alloy. The die-cast aluminum alloy of the invention has high strength and high toughness, and can obtain good mechanical properties in the as-cast state without T6 heat treatment. If T6 heat treatment is performed, the mechanical properties of the material will be further improved. The alloy material can meet the development demand of automobile lightweight and is used for manufacturing key parts such as chassis subframes and door pillars of automobile.

The heat-treatment-free die-cast alloys disclosed in the above patent publications ensure the fluidity, strength and toughness of the alloy by adding alloy elements such as Si, Mg, Cu, V, Zr, rare earth and Sr. All alloys are added with 0.01-0.06% of Sr (strontium), and the addition of Sr causes the aluminum melt to be particularly prone to gas absorption, making it difficult to ensure the purity of the melt. Even after refining and degassing, the hydrogen content still exceeds 0.18 ml/100g Al. Moreover, in large-scale industrial production, as the aluminum melt stays in the holding furnace for a long time, in the subsequent trial production of vacuum die casting, due to the high hydrogen content in the melt, there will be a large number of porosity and shrinkage defects inside different positions of the casting, making the local porosity higher than the general service requirement of <5% for die-cast parts. As a result, the elongation of the practical trial article varies significantly, and it is difficult for some regions to reach an elongation of 10% or more.

### SUMMARY OF THE DISCLOSURE

The objective of the present disclosure is to provide a heat-treatment-free high-strength and high-toughness die-cast aluminum alloy, an article manufactured therefrom and a manufacturing method therefor. The disclosure solves the problem of unstable elongation due to melt gas absorption caused by Sr element modification in such heat-treatment-free die-cast alloys, enabling the aluminum alloy die-cast part to obtain a microstructure without obvious porosity and shrinkage defects throughout the interior, thereby ensuring a tensile strength of greater than 230 MPa, a yield strength of greater than 150 MPa, and an elongation of greater than 10% at various portions of the part.

To achieve the above objective, the technical solution of the present disclosure is as follows:
A first aspect of the present disclosure provides a die-cast aluminum alloy. In addition to Al and inevitable impurity elements, the die-cast aluminum alloy comprises the following chemical components in percentage by mass: 6.5-9.5% of Si, 0.1-0.3% of Fe, 0.4-0.85% of Mn, 0.1-0.6% of Mg, 0.1-0.9% of Cu, 0.02-0.12% of Ti and 0.05-0.15% of Sb; and satisfies the following formulas: Fe+Mn ≥ 0.65% and Mn/Fe = 2.0-6.6, wherein each element symbol is substituted with the content of the corresponding element in percentage by mass.

Preferably, the die-cast aluminum alloy comprises the following chemical components in percentage by mass: 6.5-9.5% of Si, 0.1-0.3% of Fe, 0.4-0.85% of Mn, 0.1-0.6% of Mg, 0.1-0.9% of Cu, 0.02-0.12% of Ti, 0.05-0.15% of Sb, and the balance being Al and inevitable impurity elements.

Preferably, each element of the inevitable impurity elements has a content of ≤0.075% in percentage by mass, with a total content of ≤0.3%; preferably, the inevitable impurity elements contain, but not limited to, one or more of Cr, V, Ni, Sn and Zn.

Preferably, the die-cast aluminum alloy further comprises at least one of Sr, Mo and Zr, wherein Sr≤0.01%, Mo≤0.15% and Zr≤0.15%.

Preferably, the die-cast aluminum alloy comprises 0.1-0.15% of Fe; and/or 0.55-0.65% of Mn; and/or 0.1-0.4% of Mg; and/or 0.3-0.8% of Cu, and/or 0.05-0.1% of Ti; and/or 0.08-0.13% of Sb.

Preferably, the die-cast aluminum alloy of the present disclosure has a microstructure of α-Al + (α+Si) eutectic, wherein eutectic silicon is in a round granular shape with a size on submicron scale; preferably, the eutectic silicon has an average size of 0.1-1 µm, more preferably 0.54-0.76 µm.

Preferably, the microstructure of the die-cast aluminum alloy of the present disclosure does not have acicular iron-containing phase with a size greater than 20 µm and does not have pores with a size greater than 50 µm.

Preferably, the die-cast aluminum alloy of the present disclosure has a porosity of <0.5%.

Preferably, the die-cast aluminum alloy of the present disclosure has a tensile strength of greater than 230 MPa, preferably greater than 290 MPa, a yield strength of greater than 150 MPa, and an elongation of greater than 10%, preferably 13% or more.

In the composition design of the die-cast aluminum alloy of the present disclosure, the design principle of each chemical element are as follows. Herein, unless otherwise explicitly stated, all element contents are expressed in percentage by mass.

Si: Si element can significantly improve the die-casting fluidity of the aluminum alloy and improve the strength. The higher the silicon content, the more eutectic microstructure, the better the fluidity and the higher the strength, but the toughness will decrease. Therefore, the present disclosure controls the content of Si element to 6.5-9.5%, which not only ensures the fluidity of the aluminum alloy, but also reduces the proportion of eutectic silicon phase and improves the plasticity of the aluminum alloy.

Fe: The maximum solid solubility of Fe element in Al is only 0.052%. Fe element is generally treated as an impurity in wrought aluminum alloys, while in die-cast aluminum alloys, the mold release effect of Fe is almost irreplaceable in certain cases, and Fe also improves the high-temperature mechanical properties and hot cracking resistance of the alloy. However, Fe is prone to form coarse acicular β-Al5FeSi phase in die-cast aluminum alloy, leading to a decrease in strength and toughness. Therefore, the present disclosure controls the content of Fe element to 0.1-0.3%.

Mn: Mn element has little effect on the strength of the die-cast aluminum alloy, but Mn can transform the β-Al₅FeSi phase into block or Chinese-character-shaped AlFeMnSi phase, thereby improving the toughness of the alloy and the mold release of the die-cast aluminum alloy. However, an excessively high content of Mn element will form large manganese-containing phase, which affects the toughness of the alloy. For better mold release of the alloy, the sum of the Fe and Mn content is controlled to ≥0.65%. In order to improve the morphology of the iron-containing phase, the present disclosure controls the mass ratio of Mn element to Fe element to 2.0-6.6.

Mg: The addition of Mg element to the die-cast aluminum alloy can form Mg₂Si phase, which can increase the tensile strength, hardness and corrosion resistance of the aluminum alloy die-cast part. However, an excessively high Mg content will reduce the toughness and fluidity of the alloy and increase the shrinkage and hot cracking tendency of the alloy, which is particularly prominent for large-sized casting. Therefore, the present disclosure controls the content of Mg element to 0.1-0.6%.

Cu: The addition of Cu element to the die-cast aluminum alloy can form Al₂Cu phase, which can enhance the tensile strength and heat resistance of the aluminum alloy. Furthermore, the dispersed precipitated phase during the subsequent baking process further improves the strength. However, an excessively high Cu content will increase the tendency of the formation of shrinkage and hot cracking of the aluminum alloy. Therefore, the present disclosure controls the content of Cu element to 0.1-0.9%.

Ti: Ti element is used to refine the aluminum matrix and is usually added to the alloy together with B element. Fine TiB₂ and Al₃Ti phases are preferentially precipitated during the solidification process, which can act as heterogeneous nucleation site to refine grains. However, an excessive amount of Ti element will easily cause agglomeration of TiB₂ particles, affecting the toughness of the alloy. Therefore, the present disclosure controls the content of Ti element to 0.02-0.12%.

Mo: Mo element is a more effective Fe neutralizer than Mn, and can transform the β-Al₅FeSi phase into a fine α-Al(Mo,Fe)Si phase. The combined addition with Mn can completely modify both the pre-eutectic and eutectic β-Fe phases, rendering the phases uniformly and dispersedly distributed in the aluminum matrix, which can effectively hinder the movement of dislocations, improving the strength and toughness of the alloy. In order to control the cost of the alloy, the present disclosure controls the content of Mo element to ≤0.15%.

Zr: Zr element can form Al₃Zr phase in the aluminum alloy, which has a similar crystal structure to the Al₃Ti phase and a low lattice mismatch with the α-Al solid solution state, and can also refine grains. In addition, Zr can also form nano-scale dispersed phases uniformly distributed in the aluminum matrix, which can pin dislocations and improve the strength of the cast aluminum alloy at room temperature and high temperature. To control the alloy cost, the present disclosure controls the content of Zr element to ≤0.15%.

Sr: Sr element is widely used in the modification treatment of eutectic silicon in die-cast aluminum alloy. The coarse and elongated eutectic silicon can be transformed into short fibrous shape, reducing the splitting effect on the matrix and avoiding the decrease in plasticity caused by stress concentration. However, an excessively high Sr content will lead to an increase in the gas absorption of the alloy and thus the gas content in the alloy. In order to control the purity of the alloy melt so as to stably improve the elongation of the casting, the present disclosure controls the content of Sr element to ≤0.01%.

Sb: Sb element can form AlSb phase in the aluminum alloy. This phase precipitates before α-Al in the melt and promotes the nucleation and growth of α-A1. As the precipitation continues in the melt, Si phase adheres to the AlSb phase, while the α-Al grows and encapsulates the Si phase and the AlSb phase. Therefore, Sb element can effectively modify the eutectic silicon, effectively transforming the eutectic silicon from coarse flake to fine flake and even in a round granular shape. The size of eutectic silicon can reach the submicron scale (0.1-1 µm), and the aluminum matrix can be refined, making the dendritic aluminum matrix rods thinner and more uniform.

Fig. 1 shows the as-cast microstructure of a hypoeutectic Al-Si alloy with poor modification; Figs. 2 and 3 show the as-cast microstructure of a hypoeutectic Al-Si alloy modified with 0.02% Sr; Figs. 4 and 5 show the as-cast microstructure of a hypoeutectic Al-Si alloy modified with 0.1% Sb. The composition of the Al-Si alloy used in Figs. 1-5 were basically the same, wherein in addition to Al as the main component, the alloy further comprises the following in percentage by mass: 10% of Si, 0.2% of Fe, 2.1% of Cu, 0.4% of Mg and 0.02% of Ti, where the only differences were that the Al-Si alloy in Figs. 2-3 was mixed with 0.02% Sr, and the Al-Si alloy in Figs. 4-5 was mixed with 0.1% Sb.

The alloy melts in Figs. 1-5 were all manufactured by the same process below: degassing was performed at 720-730 °C with a rotary degasser. Argon with a flow rate of 4 m³/h was introduced into the degassing rotor. The rotor speed was 400 r/min, and the degassing time was 10 min. After degassing, the surface dross was skimmed off, and cast ingots with a diameter of 178 mm were obtained by semi-continuous casting. Samples were taken from the core of the cast ingots for metallographic analysis. The results show that the eutectic silicon in the circled area in Fig. 1 was poorly modified, wherein the eutectic silicon appeared as elongated strips with a size of more than 10 µm. The modification effect of the eutectic silicon in the alloy with 0.02% Sr in Figs. 2 and 3 was good, wherein the eutectic silicon was in dot shape with a maximum size of about 7 µm, but there were many pores with a size of 70-140 µm. The modification effect of eutectic silicon in the alloy with 0.1% Sb in Fig. 4 was comparable to that of the former, wherein the eutectic silicon was also distributed in dots with a maximum size of about 8 µm, but there were no pores, only slight shrinkage with shrinkage dimensions < 25 µm. The above microstructure was obtained by the semi-continuous casting process, whose cooling rate was much lower than that of die casting. After the die casting process was adopted, the size of eutectic silicon would be further refined to reach submicron scale. In addition, the Sb modification process was simple and convenient. The modification effect lasted for a long time, and the alloy modified by Sb still maintained a good modification effect even after remelting. However, an excessively high content of Sb element will produce flocculent and even coarse acicular AlSb phases, leading to a sharp decline in mechanical properties. Therefore, the present disclosure controls the content of Sb element to 0.05-0.15%.

A second aspect of the present disclosure further provides a manufacturing method for the die-cast aluminum alloy, comprising the following steps carried out in sequence:
(1) Preparing raw materials according to the chemical composition of the die-cast aluminum alloy and smelting to obtain an alloy melt, with a temperature of the alloy melt controlled at 720-730 °C;
(2) Adding a sodium-free slag remover to the melt, wherein a weight of the sodium-free slag remover accounts for 0.1-0.5% of a total weight of the alloy melt, with the temperature of the alloy melt controlled at 720-730 °C; after slag removal, adding a sodium-free covering agent to the alloy melt, wherein a weight of the sodium-free covering agent is determined according to the surface area of the alloy melt and accounts for 0.05-0.1% of the total weight of the alloy melt;
(3) Degassing the alloy melt from step (2), with the temperature of the alloy melt controlled at 720-730 °C, and skimming off surface dross; wherein the degassing is carried out under the following conditions: a mixed gas of argon and chlorine is adopted with an argon flow rate of 3.5-4.5 m³/h, a chlorine flow rate of 0.05-0.15 m³/h, and a degassing time of 10-20 min; a degassed alloy melt has a hydrogen content of ≤ 0.14 ml/100g Al;
(4) Conducting composition detection and hydrogen content detection on the degassed alloy melt, and allowing a qualified alloy melt to rest and cool to 690-720 °C to obtain the die-cast aluminum alloy.

Preferably, in step (1): required aluminum raw material is firstly charged into a melting furnace, melted and heated to 760-790 °C; then silicon, manganese, copper, antimony, molybdenum and zirconium raw materials are added and, upon complete melting, the temperature is controlled at 730-750 °C; subsequently, magnesium raw material is added and stirred until complete melting, after which the temperature is controlled at 720-730 °C; finally, titanium and strontium raw materials are added and stirred until complete melting to obtain the alloy melt, and the temperature of the alloy melt is controlled at 720-730 °C.

The iron element in the present disclosure is derived from the aluminum raw material used in the present disclosure, and presents as an impurity element in the aluminum raw material.

Preferably, in step (2): the sodium-free slag remover is added to the alloy melt by means of powder injection refining; during the powder injection refining, argon is used as a carrier, an argon flow rate is 0.1-0.3 m³/h, and a refining time is 5-10 min; both the sodium-free slag remover and the sodium-free covering agent are in powder form with a particle size of ≤ 2 mm.

Preferably, in step (3), the degassing is carried out by a rotary degasser, and a rotor speed of the rotary degasser is 400-450 r/min.

Preferably, the aluminum raw material is pure aluminum or recycled aluminum meeting the alloy composition requirement; the silicon raw material is an Al-Si master alloy, industrial silicon or fast-melting silicon; the manganese raw material is an Al-Mn master alloy or a manganese additive; the copper raw material is an Al-Cu master alloy or electrolytic copper; the antimony raw material is an Al-Sb master alloy; the molybdenum raw material is an Al-Mo master alloy; the strontium raw material is an Al-Sr master alloy; the zirconium raw material is an Al-Zr master alloy; the titanium raw material is an Al-Ti-B master alloy rod or an Al-Ti-C-B master alloy rod; the magnesium raw material is pure magnesium.

More preferably, the Al-Si master alloy is A120Si; the Al-Mn master alloy is Al10Mn; the Al-Cu master alloy is Al50Cu; the Al-Sb master alloy is Al10Sb; the Al-Mo master alloy is Al5Mo; the Al-Sr master alloy is Al10Sr; the Al-Zr master alloy is Al10Zr; the Al-Ti-B master alloy is Al5TiB; the Al-Ti-C-B master alloy is A12Ti0.2C0.2B.

In the manufacturing method for the above die-cast aluminum alloy of the present disclosure:
When rotary degassing is carried out by a rotary degasser, a mixed gas of argon and chlorine is adopted with an argon flow rate of 3.5-4.5 m³/h, a chlorine flow rate of 0.05-0.15 m³/h, and a degassing time of 10-20 min. The present disclosure improves the degassing performance by mixing a small amount of chlorine into argon as the degassing medium, utilizing the adsorption of hydrogen by dispersed argon bubbles in the melt and the chemical reaction between chlorine gas and hydrogen in the melt, thereby controlling the hydrogen content in the alloy melt to ≤ 0.14 ml/100g Al.

The removal of hydrogen from the molten aluminum alloy is achieved by the reaction of hydrogen atoms to generate hydrogen gas, which is then transferred to the gas phase. The reaction process is controlled by the hydrogen partial pressure difference between the melt and the gas phase. When the hydrogen partial pressure in the melt is higher than that in the gas phase, hydrogen gas is released from the melt. Argon is introduced into the melt, the hydrogen partial pressure in the argon bubbles is lower than that in the melt, and the hydrogen in the melt diffuses into the argon bubbles to generate hydrogen gas, which is carried out of the melt as the argon bubbles float up.

In the degassing step, the argon gas flowing out from the rotor outlet is broken into very fine bubbles by the high-speed rotation of the rotor in the rotary degasser, which increases the surface area and dispersion degree of the bubbles in the melt, so that the argon bubbles are more fully in contact with hydrogen atoms in the melt, and thus the degassing efficiency is improved. The bubble breaking and dispersion level in the degassing process depend on the speed of the rotor. The higher the rotor speed, the better the bubble breaking and dispersion level, and the better the degassing result. However, an excessively high rotational speed leads to equipment instability and will easily cause rotor fracture and failure. An excessively low rotational speed results in excessively large bubbles in the melt, which would limit the range of influence to a small area around the rotor. The bubbles will float up rapidly in the melt with a short residence time, leading to poor effect of hydrogen capture. Therefore, the present disclosure controls the rotor speed at 400-450 r/min.

The flow rate of argon introduced into the rotor is related to the rotor speed. An excessively low argon flow rate results in a small number of bubbles in the melt, and an excessively high argon flow rate results in the rotor being unable to fully break and disperse the bubbles. The excess bubbles cause the fine bubbles to reaggregate into large bubbles, which float up near the rotor and cause the liquid surface to churn, resulting in a decrease in degassing efficiency. Therefore, the argon flow rate is controlled at 3.5-4.5 m³/h in the present disclosure.

The present disclosure enhances the degassing capacity by adding a small amount of chlorine to argon, utilizing the reaction of chlorine in the melt, which mainly undergoes the following reactions: Cl₂+H₂=2HCl↑ and 2Al+3Cl₂=2AlCl₃↑. Chlorine directly reacts with hydrogen to remove hydrogen, while AlCl₃ and HCl generated by the reaction of chlorine with aluminum float up in the melt as gas state, also providing the adsorption degassing effect. However, since chlorine directly reacts with Al, an excessive amount of chlorine will lead to slag formation in the melt. Therefore, the chlorine flow rate is controlled at 0.05-0.15 m³/h in the present disclosure.

Argon is introduced by rotary degassing into the melt to adsorb hydrogen in the melt, and it is necessary to control the hydrogen content of a large amount of melt at a low level, thus sufficient degassing time must be ensured. An excessively short degassing time will obviously lead to incomplete degassing. After a continuous decrease of the hydrogen content in the melt, an equilibrium is reached, therefore an excessively long degassing time cannot further reduce the hydrogen content in the melt, but instead causes slag formation and oxidation of the melt. Thus, the degassing time is controlled at 10-20 min in the present disclosure.

The sodium-free slag remover and the sodium-free covering agent used in the present disclosure is not particularly limited, and those commonly used in the art can be used. For example, the sodium-free slag remover includes, but not limited to, the following components in percentage by mass: 42% of KCl, 46% of MgCl₂, 6% of BaCl₂ and 6% of CaF₂; the sodium-free covering agent includes, but not limited to, the following components in percentage by mass: 80% of (KCl + MgCl₂) and 20% of CaF₂.

The qualified alloy melt in the present disclosure refers to an alloy melt having the above composition according to the present disclosure with a hydrogen content of ≤ 0.14 ml/100g Al.

A third aspect of the present disclosure provides an article prepared from the above die-cast aluminum alloy, such as an aluminum alloy die-cast part. The aluminum alloy die-cast part can be an automobile component.

Compared with the prior art, the advantages of the present disclosure are as follows:
1. Sr element is generally added in the conventional alloy to modify the eutectic silicon. Sr will reduce the liquid phase filling capacity of the alloy during solidification, thus easily causing shrinkage cavity and shrinkage defects. In order to ensure the modification effect of eutectic Si, the addition amount of Sr is usually 0.02%. However, high Sr content leads to serious gas absorption of the alloy melt, and thus it is hard for the conventional degassing process in the die-casting industry to control the hydrogen content of the melt to 0.18 ml/100g Al or less, resulting in more porosity and shrinkage defects during subsequent vacuum die cast of parts. Some porosity and shrinkage can reach a size to 100 µm or more.
   The heat-treatment-free die-cast aluminum alloy of the present disclosure adds Sb element to replace Sr element for the first time to modify the eutectic silicon, which can effectively address the problem of high hydrogen content caused by gas absorption of the melt with high Sr content, thus addressing the problem of coarse acicular eutectic silicon in the alloy microstructure that seriously deteriorates the mechanical properties of the die-cast aluminum alloy for hypoeutectic Al-Si-based die-cast aluminum alloy.
2. The aluminum alloy of the present disclosure modifies the eutectic silicon by adding Sb element, which can effectively transform the eutectic silicon from coarse flake to fine flake and even in a round granular shape, reaching the submicron scale (0.1-1 µm). The aluminum matrix can be refined, making the dendritic aluminum matrix rods thinner. Compared with adding Ti element alone in the prior art, the composite refinement effect is better, and the dendrites of the aluminum matrix are uniformly distributed, thus significantly improving the mechanical properties, especially the elongation.
3. The aluminum alloy of the present disclosure adopts Sb element for modification and refinement. The process is simple and convenient, and the modification effect lasts for a long time. The alloy can retain a good modification effect and does not need for re-treatment even when remelting, while the Sr element modification process is relatively complex, because Sr is easy to volatilize in the high-temperature melt, leading to lower yield after addition, so that Sr element needs to be added again when remelting the alloy.
4. The present disclosure improves the morphology of the iron-containing phase and the mechanical properties and mold release of the alloy by controlling the total content and ratio of Fe and Mn elements.
5. In the melt degassing process of the manufacturing method of the present disclosure, a mixed gas of argon and chlorine is adopted as the degassing medium in the heat-treatment-free die-cast aluminum alloy for the first time, which improves the melt degassing efficiency, ensuring that the hydrogen content in the melt can be controlled to 0.14 ml/100g Al or less, providing a prerequisite for vacuum die-casting components with low porosity, and thus stably improves the elongation of the components.

### BRIEF DESCRIPTION OF THE DRAWINGS

Fig. 1 is a photograph showing the as-cast microstructure of a hypoeutectic Al-Si alloy with poor modification;
Fig. 2 is a photograph showing the as-cast microstructure of a hypoeutectic Al-Si alloy modified with 0.02% Sr;
Fig. 3 is an enlarged photograph showing the as-cast microstructure of a hypoeutectic Al-Si alloy modified with 0.02% Sr;
Fig. 4 is a photograph showing the as-cast microstructure of a hypoeutectic Al-Si alloy modified with 0.1% Sb;
Fig. 5 is an enlarged photograph showing the as-cast microstructure of a hypoeutectic Al-Si alloy modified with 0.1% Sb;
Fig. 6 is a photograph showing a typical metallographic microstructure of the cross section of a vacuum die-cast test piece in Example 5 according to the present disclosure;
Fig. 7 is an enlarged photograph showing a typical metallographic microstructure of the cross section of a vacuum die-cast test piece in Example 5 according to the present disclosure;
Fig. 8 is a photograph showing a typical metallographic microstructure of the cross section of a vacuum die-cast test piece in Comparative Example 1.

### DETAILED DESCRIPTION

The present disclosure will be described in further detail below in conjunction with specific embodiments and the accompanied drawings. It should be understood that the specific embodiments described herein are only used for illustration of the present disclosure and do not limit the present disclosure.

The property parameters of the present disclosure were measured as follows, respectively.

Chemical composition of the alloy melt was determined by an ARL 4460 direct-reading spectrometer.

Hydrogen content in the alloy melt was determined by an ABB-Alscan hydrogen analyzer.

Tensile strength, yield strength and elongation of the die-cast aluminum alloy were determined by an AG-xPlus-100kN electronic universal testing machine.

Microstructure of the die-cast aluminum alloy was observed and photographed by a Leica Sereozoom S9i metallographic microscope.

Average size of eutectic silicon particles in the microstructure of the die-cast aluminum alloy was determined based on scanning electron microscope photographs, wherein the size and number of eutectic silicon particles were identified using ImageJ software, and the average size was determined.

Porosity of the die-cast aluminum alloy was determined based on metallographic photographs, with the area of pores identified using ImageJ software, and the proportion of the area calculated.

The compositions of the aluminum alloys of the Examples and Comparative Examples of the present disclosure are shown in Table 1, with the balance comprising Al and inevitable impurity elements. The manufacturing process parameters for the Examples and Comparative Examples of the present disclosure are shown in Table 2. The properties of the Examples and Comparative Examples of the present disclosure are shown in Table 3.

### Example 1

The heat-treatment-free high-strength and high-toughness die-cast aluminum alloy of Example 1 comprised the following chemical components in percentage by mass: 6.56% of Si, 0.22% of Fe, 0.45% of Mn, 0.38% of Mg, 0.9% of Cu, 0.08% of Ti, 0.15% of Sb, and the balance being Al and inevitable impurity elements. In the inevitable impurity elements, the content of each element was ≤0.075%, and the total content was ≤0.3%. The manufacturing method included:
(1) preparing pure aluminum, pure Mg, Al20Si, Al10Mn, Al50Cu, Al10Sb and Al2Ti0.2C0.2B raw materials according to the above chemical composition of the die-cast aluminum alloy in percentage by mass, preheating and drying the raw materials to remove moisture;
(2) charging the required aluminum raw material into a smelting furnace, melting and heating to 770 °C, wherein the iron element was introduced through the aluminum raw material and was present as an impurity of the aluminum raw material; then adding Al20Si, Al10Mn, Al50Cu and Al10Sb, wherein the temperature was controlled at 740 °C after raw materials were completely melted; next, adding Mg raw material and stirring, wherein the temperature was controlled at 730 °C after the raw material was completely melted; subsequently adding Al2Ti0.2C0.2B and stirring to obtain alloy melt upon complete melting of raw materials, wherein the temperature of the obtained alloy melt was controlled at 730 °C;
(3) Conducting composition detection on the alloy melt, and upon composition qualified, adding a sodium-free slag remover to the melt by means of powder injection refining, wherein the weight of the sodium-free slag remover accounted for 0.2% of the total weight of the alloy melt, and the temperature of the alloy melt was controlled at 730 °C; after slag removal, adding a sodium-free covering agent to the alloy melt, wherein the weight of the sodium-free covering agent was determined according to the surface area of the melt and accounted for about 0.05% of the total weight of the alloy melt; wherein during the powder injection refining, argon was used as a carrier with an argon flow rate of 0.1 m³/h, and a refining time was 10 min; and wherein both the sodium-free slag remover and the sodium-free covering agent were in powder form with a particle size of ≤ 2 mm;
(4) Degassing the alloy melt by a rotary degasser, with the temperature of the alloy melt controlled at 730 °C, and skimming off surface dross, wherein the degassing was carried out under the following conditions: a rotor speed of 400 r/min, using a mixed gas of argon and chlorine with an argon flow rate of 3.5 m³/h, a chlorine flow rate of 0.05 m³/h, and a degassing time of 10 min;
(5) Conducting composition detection and hydrogen content detection on the refined and degassed alloy melt, and allowing the qualified alloy melt to rest and cool to 690 °C to obtain the heat-treatment-free high-strength and high-toughness die-cast aluminum alloy, wherein the alloy melt was determined to be qualified when: the composition of the alloy melt met the requirements of the present disclosure, and the hydrogen content of the alloy melt determined by the ABB-Alscan hydrogen analyzer was ≤ 0.14 ml/100g Al.

Subsequently, the heat-treatment-free die-cast aluminum alloy was prepared into tensile test bars or die-cast test pieces by vacuum die casting for corresponding property test. The die-casting temperature was 690 °C, the mold temperature was 200 °C, the injection velocity was 2.5 m/s, the casting pressure was 65 MPa, and the vacuum degree was 200 mbar.

### Examples 2-9

The heat-treatment-free die-cast aluminum alloys of Examples 2-9 were manufactured by the method basically the same as that in Example 1, except that the aluminum alloy composition and manufacturing process parameters were adjusted within the ranges defined by the present disclosure, which are specifically shown in Table 1 and Table 2. Unless otherwise specified, the molybdenum raw material in Examples 7-9 was Al5Mo, the strontium raw material was Al10Sr, and the zirconium raw material was Al10Zr.

### Comparative Example 1

The heat-treatment-free die-cast aluminum alloy of Comparative Example 1 comprised the following components in percentage by mass: 8.02% of Si, 0.18% of Fe, 0.47% of Mn, 0.36% of Mg, 0.49% of Cu, 0.11% of Ti, 0.025% of Sr, the balance being Al and inevitable impurity elements. In the inevitable impurity elements, the content of each element was ≤ 0.075%, and the total content was ≤ 0.3%. The manufacturing method included:
(1) Preparing pure aluminum, pure Mg, Al20Si, Al50Cu, Al10Mn, Al10Sr and Al2Ti0.2C0.2B according to the above alloy composition in percentage by mass, preheating and drying the raw materials to remove moisture;
(2) charging the required aluminum raw material into a smelting furnace, melting and heating to 770 °C, wherein the iron element was introduced through the aluminum raw material and was present as an impurity of the aluminum raw material; then adding Al20Si, Al50Cu and Al10Mn, wherein the temperature was controlled at 740 °C after raw materials were completely melted; next, adding Mg raw material and stirring, wherein the temperature was controlled at 730 °C after the raw material was completely melted; finally adding Al2Ti0.2C0.2B and Al10Sr and stirring to obtain alloy melt upon complete melting of raw materials, wherein the temperature of the obtained alloy melt was controlled at 730 °C;
(3) Conducting composition detection on the alloy melt, and upon composition qualified, adding a sodium-free slag remover to the melt by means of powder injection refining, wherein the weight of the sodium-free slag remover accounted for 0.3% of the total weight of the alloy melt, and the temperature of the alloy melt was controlled at 725 °C; after slag removal, adding a sodium-free covering agent to the alloy melt, wherein the weight of the sodium-free covering agent was determined according to the surface area of the melt and accounted for about 0.1% of the total weight of the alloy melt; wherein during the powder injection refining, argon was used as a carrier with an argon flow rate of 0.12 m³/h, and a refining time was 9.5 min; and wherein both the sodium-free slag remover and the sodium-free covering agent were in powder form with a particle size of ≤ 2 mm;
(4) Degassing the alloy melt by a rotary degasser, with the temperature of the alloy melt controlled at 728 °C, and skimming off surface dross, wherein the degassing process was carried out under the following conditions: a rotor speed of 425 r/min, using a mixed gas of argon and chlorine with an argon flow rate of 4 m³/h, a chlorine flow rate of 0.08 m³/h, and a degassing time of 15 min;
(5) Conducting composition detection on the refined and degassed alloy melt, and allowing the qualified alloy melt to rest and cool to 695°C to obtain the heat-treatment-free die-cast aluminum alloy.

Subsequently, the heat-treatment-free die-cast aluminum alloy was prepared into tensile test bars or die-cast test pieces by vacuum die casting for corresponding property test. The die-casting temperature was 690 °C, the mold temperature was 200 °C, the injection velocity was 2.5 m/s, the casting pressure was 65 MPa, and the vacuum degree was 200 mbar.

### Comparative Example 2

Comparative Example 2 was manufactured by the method basically the same as that in Example 1 of the present disclosure in terms of aluminum alloy composition and manufacturing method, except that the total content and ratio of Fe and Mn did not meet the requirement of the present disclosure, which are specifically shown in Table 1 and Table 2.

### Comparative Example 3

Comparative Example 3 was manufactured by the method basically the same as that in Example 1 of the present disclosure in terms of aluminum alloy composition and manufacturing method, except that the Cu content was 1.00%, which are specifically shown in Table 1 and Table 2.

**Table 1 (unit: mass percentage)**

| | Si | Fe | Mn | Mg | Cu | Ti | Sb | Sr | Mo | Zr | Fe+Mn | Mn/Fe |
|---|---|---|---|---|---|---|---|---|---|---|---|---|
| Example 1 | 6.56 | 0.22 | 0.45 | 0.38 | 0.90 | 0.09 | 0.15 | - | - | - | 0.67 | 2.05 |
| Example 2 | 9.50 | 0.12 | 0.57 | 0.40 | 0.30 | 0.08 | 0.12 | - | - | - | 0.69 | 4.75 |
| Example 3 | 8.12 | 0.30 | 0.84 | 0.55 | 0.60 | 0.12 | 0.13 | - | - | - | 1.14 | 2.80 |
| Example 4 | 8.07 | 0.20 | 0.48 | 0.20 | 0.10 | 0.02 | 0.14 | - | - | - | 0.68 | 2.40 |
| Example 5 | 7.61 | 0.15 | 0.61 | 0.35 | 0.48 | 0.04 | 0.10 | - | - | - | 0.76 | 4.07 |
| Example 6 | 8.10 | 0.13 | 0.85 | 0.60 | 0.50 | 0.10 | 0.09 | - | - | - | 0.98 | 6.54 |
| Example 7 | 7.59 | 0.16 | 0.56 | 0.10 | 0.38 | 0.07 | 0.05 | - | 0.10 | - | 0.72 | 3.50 |
| Example 8 | 8.02 | 0.17 | 0.54 | 0.32 | 0.20 | 0.06 | 0.11 | - | 0.11 | 0.06 | 0.71 | 3.18 |
| Example 9 | 7.48 | 0.14 | 0.63 | 0.28 | 0.80 | 0.05 | 0.08 | 0.0096 | 0.12 | 0.04 | 0.77 | 4.50 |
| Comparative Example 1 | 8.02 | 0.18 | 0.47 | 0.36 | 0.49 | 0.11 | - | 0.0250 | - | - | 0.65 | 2.61 |
| Comparative Example 2 | 6.56 | 0.29 | 0.38 | 0.38 | 0.90 | 0.09 | 0.15 | - | - | - | 0.74 | 1.55 |
| Comparative Example 3 | 6.56 | 0.22 | 0.45 | 0.38 | 1.00 | 0.09 | 0.15 | - | - | - | 0.67 | 2.05 |

**Table 2**

| | Melt temperature °C | Weight percentage of sodium-free slag remover % | Weight percentage of sodium-free covering agent % | Argon flow rate during refining m³/h | Refining time min | Melt temperature during degassing °C | Rotor speed r/min | Argon flow rate during degassing m³/h | Chlorine flow rate during degassing m³/h | Degassing time min | Rest and cooling temperature °C |
|---|---|---|---|---|---|---|---|---|---|---|---|
| Example 1 | 730 | 0.20 | 0.05 | 0.10 | 10 | 730 | 400 | 3.5 | 0.05 | 10 | 690 |
| Example 2 | 727 | 0.25 | 0.06 | 0.15 | 9.0 | 725 | 435 | 4.5 | 0.075 | 12 | 693 |
| Example 3 | 729 | 0.10 | 0.07 | 0.21 | 6.0 | 720 | 420 | 3.6 | 0.085 | 13 | 692 |
| Example 4 | 724 | 0.15 | 0.10 | 0.30 | 5.0 | 724 | 430 | 4.3 | 0.125 | 20 | 694 |
| Example 5 | 728 | 0.35 | 0.09 | 0.20 | 6.5 | 729 | 450 | 3.8 | 0.15 | 16 | 705 |
| Example 6 | 720 | 0.40 | 0.085 | 0.23 | 8.0 | 726 | 415 | 4.4 | 0.11 | 17 | 720 |
| Example 7 | 726 | 0.45 | 0.08 | 0.25 | 7.5 | 722 | 440 | 4.1 | 0.06 | 14 | 710 |
| Example 8 | 723 | 0.50 | 0.095 | 0.18 | 7.0 | 721 | 410 | 4.2 | 0.065 | 18 | 705 |
| Example 9 | 721 | 0.38 | 0.065 | 0.17 | 8.5 | 727 | 405 | 3.9 | 0.12 | 19 | 697 |
| Comparative Example 1 | 725 | 0.30 | 0.10 | 0.12 | 9.5 | 728 | 425 | 4 | 0.08 | 15 | 695 |
| Comparative Example 2 | 730 | 0.20 | 0.05 | 0.10 | 10 | 730 | 400 | 3.5 | 0.05 | 10 | 690 |
| Comparative Example 3 | 730 | 0.20 | 0.05 | 0.10 | 10 | 730 | 400 | 3.5 | 0.05 | 10 | 690 |

**Table 3**

| | Average size of eutectic silicon µm | Tensile strength MPa | Yield strength MPa | Elongation % | Porosity % |
|---|---|---|---|---|---|
| Example 1 | 0.67 | 295 | 170 | 14.0 | 0.28 |
| Example 2 | 0.54 | 305 | 185 | 13.8 | 0.34 |
| Example 3 | 0.62 | 298 | 178 | 14.1 | 0.25 |
| Example 4 | 0.61 | 312 | 181 | 14.6 | 0.33 |
| Example 5 | 0.76 | 299 | 168 | 13.6 | 0.21 |
| Example 6 | 0.66 | 303 | 162 | 13.7 | 0.45 |
| Example 7 | 0.75 | 294 | 165 | 13.8 | 0.42 |
| Example 8 | 0.64 | 300 | 172 | 13.5 | 0.31 |
| Example 9 | 0.72 | 303 | 166 | 13.2 | 0.29 |
| Comparative Example 1 | 0.82 | 295 | 157 | 8.7 | 5.21 |
| Comparative Example 2 | 0.66 | 297 | 160 | 8.5 | 0.41 |
| Comparative Example 3 | 0.83 | 315 | 185 | 8.2 | 0.39 |

The comparison results of the mechanical properties and average size of the eutectic silicon of the die-cast test pieces prepared from the aluminum alloys according to the present disclosure and those prepared from the comparative alloys are shown in Table 3. The photographs showing the microstructures of Example 5 and Comparative Example 1 are presented in Figs. 6, 7 and 8.

Figs. 6 and 7 are the typical optical micrographs of the cross section of the die-cast test piece in Example 5 obtained by an optical microscope. The results indicated that the microstructure of the aluminum alloy material of Example 5 was α-Al + (α+Si) eutectic, with a fine and uniform internal microstructure and did not had coarse acicular iron-containing phase larger than 20 µm in size. The eutectic silicon modification effect was good. The eutectic silicon was in dot shape with a size of less than 1 µm (the average size of eutectic silicon particles in Fig. 7 calculated by ImageJ software was 0.76 µm, reaching the submicron scale). In addition, there were no pores larger than 50 µm inside the material, only slight shrinkage porosity (porosity < 0.5%), thus ensuring a high elongation for the Examples.

Fig. 8 is a typical optical micrograph of the cross section of the die-cast test piece in Comparative Example 1. The results indicated that the internal microstructure of the material was fine and uniform and did not have coarse acicular iron-containing phases larger than 20 µm in size. The eutectic silicon modification effect was also good. The average size of eutectic silicon particles was 0.82 µm, also reaching the submicron scale. However, there were obvious pore defects larger than 50 µm in size, which led to reduction of elongation.

It can be seen from Table 3 that the die-cast test pieces of the Examples of the present disclosure exhibited a tensile strength of more than 290 MPa, a yield strength of more than 150 MPa, and an elongation of 13% or more. Although the die-cast test pieces of Comparative Examples 1, 2 and 3 met the strength requirements, their elongations were only 8.7%, 8.5% and 8.2%, respectively.

In summary, the present disclosure has achieved an excellent eutectic silicon modification effect by adopting the Sb element modification/refinement process combined with the optimization of alloy composition (e.g., controlling the total content and ratio of Fe and Mn, as well as the Cu content), which can effectively address the problem of high hydrogen content caused by gas absorption of the melt with high Sr content. Combined with the rotary degassing process, the hydrogen content of the alloy was controlled to 0.14 ml/100g Al or less. After die casting, the internal microstructure was fine and uniform and did not had coarse acicular iron-containing phase larger than 20 µm in size. The eutectic silicon was in a round granular shape with an size reaching submicron scale, and there were no obvious porosity and shrinkage larger than 50 µm in size. The alloy can obtain excellent mechanical properties with an as-cast yield strength of more than 150 MPa, a porosity of below 0.5%, and an elongation of 13% or more, suitable for the manufacture of large integrated automobile components via vacuum die casting. Such large integrated automobile components can not only meet the industry application requirement for automobile components (porosity < 5% and elongation of more than 10%) but also satisfy the requirement for subsequent assembly.

It should be noted that all technical features described in the present application may be combined or incorporated in any manner, unless contradicts with each other. As will be apparent to those skilled in the art, various modifications and variations may be made to the present disclosure without departing from the spirit and scope thereof. For instance, features illustrated or described as part of one embodiment may be employed in conjunction with another embodiment to yield further embodiments. Accordingly, the present disclosure is intended to embrace all such modifications and variations that fall within the scope of the appended claims and their equivalents.

## Claims

1. A die-cast aluminum alloy, in addition to Al and inevitable impurity elements, comprising the following chemical components in percentage by mass: 6.5-9.5% of Si, 0.1-0.3% of Fe, 0.4-0.85% of Mn, 0.1-0.6% of Mg, 0.1-0.9% of Cu, 0.02-0.12% of Ti and 0.05-0.15% of Sb; and satisfying the following formulas: Fe+Mn ≥ 0.65% and Mn/Fe = 2.0-6.6, wherein each element symbol is substituted with the content of the corresponding element in percentage by mass.

2. The die-cast aluminum alloy according to claim 1, wherein the die-cast aluminum alloy comprises the following chemical components in percentage by mass: 6.5-9.5% of Si, 0.1-0.3% of Fe, 0.4-0.85% of Mn, 0.1-0.6% of Mg, 0.1-0.9% of Cu, 0.02-0.12% of Ti, 0.05-0.15% of Sb, and the balance being Al and inevitable impurity elements.

3. The die-cast aluminum alloy according to claim 1 or 2, wherein each element of the inevitable impurity elements has a content of ≤0.075% in percentage by mass, with a total content of ≤0.3%; preferably, the inevitable impurity elements contain one or more of Cr, V, Ni, Sn and Zn.

4. The die-cast aluminum alloy according to any one of claims 1 to 3, wherein the die-cast aluminum alloy further comprises at least one of Sr, Mo and Zr, wherein Sr≤0.01%, Mo≤0.15% and Zr≤0.15%.

5. The die-cast aluminum alloy according to any one of claims 1 to 4, wherein the die-cast aluminum alloy comprises 0.1-0.15% of Fe; and/or 0.55-0.65% of Mn; and/or 0.1-0.4% of Mg; and/or 0.3-0.8% of Cu, and/or 0.05-0.1% of Ti; and/or 0.08-0.13% of Sb.

6. The die-cast aluminum alloy according to any one of claims 1 to 5, wherein the die-cast aluminum alloy has a microstructure of α-Al + (α+Si) eutectic, wherein eutectic silicon is in a round granular shape with a size on submicron scale; preferably, the eutectic silicon has an average size of 0.1-1 µm, more preferably 0.54-0.76 µm; preferably, the microstructure of the die-cast aluminum alloy does not have acicular iron-containing phase with a size greater than 20 µm and does not have pores with a size greater than 50 µm; preferably, the die-cast aluminum alloy has a porosity of <0.5%.

7. The die-cast aluminum alloy according to any one of claims 1 to 6, wherein the die-cast aluminum alloy has a tensile strength of greater than 230 MPa, preferably greater than 290 MPa, a yield strength of greater than 150 MPa, and an elongation of greater than 10%, preferably 13% or more.

8. A manufacturing method for the die-cast aluminum alloy according to any one of claims 1 to 7, comprising the following steps carried out in sequence:
(1) Preparing raw materials according to the chemical composition of the die-cast aluminum alloy and smelting to obtain an alloy melt, with a temperature of the alloy melt controlled at 720-730 °C;
(2) Adding a sodium-free slag remover to the alloy melt, wherein a weight of the sodium-free slag remover accounts for 0.1-0.5% of a total weight of the alloy melt, with the temperature of the alloy melt controlled at 720-730 °C; after slag removal, adding a sodium-free covering agent to the alloy melt, wherein a weight of the sodium-free covering agent accounts for 0.05-0.1% of the total weight of the alloy melt;
(3) Degassing the alloy melt from step (2), with the temperature of the alloy melt controlled at 720-730 °C, and skimming off surface dross; wherein the degassing is carried out under the following conditions: a mixed gas of argon and chlorine is adopted with an argon flow rate of 3.5-4.5 m³/h, a chlorine flow rate of 0.05-0.15 m³/h, and a degassing time of 10-20 min; a degassed alloy melt has a hydrogen content of ≤ 0.14 ml/100g Al;
(4) Conducting composition detection and hydrogen content detection on the degassed alloy melt, and allowing a qualified alloy melt to rest and cool to 690-720 °C to obtain the die-cast aluminum alloy.

9. The manufacturing method according to claim 8, wherein in step (1): required aluminum raw material is firstly charged into a melting furnace, melted and heated to 760-790 °C; then silicon, manganese, copper, antimony, molybdenum and zirconium raw materials are added and, upon complete melting, the temperature is controlled at 730-750 °C; subsequently, magnesium raw material is added and stirred until complete melting, after which the temperature is controlled at 720-730 °C; finally, titanium and strontium raw materials are added and stirred until complete melting to obtain the alloy melt, and the temperature of the alloy melt is controlled at 720-730 °C.

10. The manufacturing method according to claim 8, wherein in step (2), the sodium-free slag remover is added to the alloy melt by means of powder injection refining; during the powder injection refining, argon is used as a carrier with an argon flow rate of 0.1-0.3 m³/h, and a refining time is 5-10 min; both the sodium-free slag remover and the sodium-free covering agent are in powder form with a particle size of ≤ 2 mm.

11. The manufacturing method according to claim 8, wherein in step (3), the degassing is carried out by a rotary degasser, and a rotor speed of the rotary degasser is 400-450 r/min.

12. The manufacturing method according to claim 9, wherein the aluminum raw material is pure aluminum or recycled aluminum meeting the alloy composition requirement; the silicon raw material is an Al-Si master alloy, industrial silicon or fast-melting silicon; the manganese raw material is an Al-Mn master alloy or a manganese additive; the copper raw material is an Al-Cu master alloy or electrolytic copper; the antimony raw material is an Al-Sb master alloy; the molybdenum raw material is an Al-Mo master alloy; the strontium raw material is an Al-Sr master alloy; the zirconium raw material is an Al-Zr master alloy; the titanium raw material is an Al-Ti-B master alloy rod or an Al-Ti-C-B master alloy rod; the magnesium raw material is pure magnesium.

13. The manufacturing method according to claim 12, wherein the Al-Si master alloy is Al20Si; the Al-Mn master alloy is Al10Mn; the Al-Cu master alloy is Al50Cu; the Al-Sb master alloy is Al10Sb; the Al-Mo master alloy is Al5Mo; the Al-Sr master alloy is Al10Sr; the Al-Zr master alloy is All0Zr; the Al-Ti-B master alloy is Al5TiB; the Al-Ti-C-B master alloy is Al2Ti0.2C0.2B.

14. An article manufactured from the die-cast aluminum alloy according to any one of claims 1 to 7, wherein the article is an aluminum alloy die-cast part.

15. The article according to claim 14, wherein the aluminum alloy die-cast part is an automobile component.
